

## UNITED STATES PATENT OFFICE

2,605,182

DIAZOTYPES CONTAINING N-SUBSTITUTED  
P-DIAZOANILINES HAVING RADICALS OF  
AT LEAST FOUR CONJUGATED C—C DOU-  
BLE BONDS AS N-SUBSTITUENTS

Willard D. Peterson, Easton, Pa., assignor to General Aniline &amp; Film Corporation, New York, N. Y., a corporation of Delaware

No Drawing. Application November 28, 1947,  
Serial No. 788,656

4 Claims. (Cl. 95—7)

1

This invention relates to diazotype reproducing material which will reproduce positive copies from positive originals, and more particularly to the use of diazo compounds in said diazotype materials as the light sensitive element which will decompose under exposure to long wave length light.

In the reproduction of positive copies from positive originals by the diazotype method diazo compounds have been employed which will be decomposed most effectively by light in the range of 3600 Å. to 4200 Å. The diazo compounds which have thus been employed have not been selected because of this sensitivity to that range of light emanations, but have been selected because they possess other properties which particularly suit them for use in the diazotype process. Thus these diazos will couple with azo dye coupling components in the proper coupling medium or atmosphere to produce dye images in a wide range of colors, particularly in deep shades. They also can be incorporated together with the coupling component in a two-component diazotype system and stored for reasonable lengths of time without danger of coupling taking place prior to exposure and development. They will also, under proper conditions, produce wash-fast images which will not bleed to any appreciable extent. Those diazo compounds which have been found to possess these properties requisite for efficient diazotype reproduction embrace for the most part monodiazoo derivatives of p-phenylene-diamines wherein the undiazotized amino group may be substituted by simple substituents such as alkyl, alkylol, phenyl and substituted phenyl and the like. Diazo derivatives of o-amino naphthols have also been employed to some extent and monodiazoo derivatives of o-phenyldiamines where the undiazotized amino group is at least mono-substituted by one of the above-mentioned substituent groups have been suggested, but are of little importance commercially. These diazo compounds which have been found most suitable for diazotype reproduction work as indicated above are most effectively decomposed by sources of light emitting rays in the 3600 Å. to 4200 Å. line. In general, it can be said that diazotype materials heretofore employed are decomposed only by wave length of light shorter than 4800—5000 Å.

In order to meet the light requirements of these diazotype materials and of other photoprinting materials such as blueprints, and silver salt sensitized photo materials such as so-called Van Dyke paper, it has been necessary to confine

2

exposure equipment to sources of light which are rich in emanations of rays having wave lengths in the 3600—4200 Å. range. When using incandescent lamps as the light source in order to produce a sufficient concentration of such rays, it is necessary to operate the incandescent lamps at higher voltage than bulb life considerations permit. Since incandescent lamps emit light which is particularly rich in wave lengths above the 4000 Å. line they constitute a wasteful source of energy for this purpose. Until the advent of the high pressure mercury-quartz-arc lamp which efficiently emits light rich in wave lengths within the 3600—4200 Å. range, exposure devices for diazotypes and other photoprinting materials having the same light sensitive characteristics made use of carbon-arc lamps and low pressure mercury vapor tubes which have definite operational disadvantages. The high pressure quartz-mercury vapor arc lamps having high ultraviolet output operate at approximately 75 watts per inch and require bulky and expensive accessories for operation. Other sources of light of recent development such as fluorescent lights could be more effectively adapted to exposure equipment for diazotype and similar photoprinting reproduction, and would lend themselves to simpler and less expensive operation. However, such light sources have heretofore been rejected because of the low output of light emanations in the necessary range for efficient photo decompositions of the diazo or other light sensitive compound.

It has now been discovered that a new class of diazo compounds not heretofore employed for diazotype or photosensitive printing may be effectively employed in diazotypes and efficiently decomposed by light having longer wave lengths such as 5200—6000 Å. These are wave lengths of light which are principally emitted by fluorescent lamps, incandescent photoflood and other types of incandescent lamps. Consequently, when using such diazo compounds as the light sensitive element of the photo reproduction material the exposure may be carried out by using equipment containing fluorescent lights which may be a simple portable lamp or a portable unit containing incandescent photoflood lamps, thus making possible efficient exposure of a photoprinting material by a small user who is limited to portable, easily operated units. The new class of diazo compounds will also decompose efficiently upon exposure to presently used sources of light which operate most efficiently in the shorter wave length ranges,

such as the 3600-4200 Å. range, to which present diazotype materials are most sensitive.

The new class of diazo compounds may be defined as N-substituted p-diazoanilines in which the substituent or substituents on the amino group contain at least four conjugated carbon to carbon bonds in a cyclic nucleus. The diazo compounds of this class are diazo derivatives of amines which may be represented by the formulae:



and



wherein  $R_1$  contains at least four conjugated carbon to carbon double bonds in an aromatic or heterocyclic ring system,  $R_2$  is a heterocyclic ring system containing the N atom as a hetero atom and R may be hydrogen, alkyl, such as methyl, ethyl and butyl, and substituted alkyl, such as carboxymethyl; wherein Y represents hydrogen or acylamino, such as acetamino, benzamido; alkyl, such as methyl and ethyl; carboxyl, such as sulfoxy; and alkoxy, such as methoxy and ethoxy; and wherein X represents a negative ion such as chloride or a complex group acting as stabilizer for the diazo compound, such as, boron trifluoride, zinc chloride, cadmium chloride, naphthalene disulfonic acid, and the like.

Diazo compounds of this class can be readily prepared by the diazotization of the corresponding amine and the formation of the diazo complex by the usual methods. The amines may be prepared by one of the following methods.

(1) reaction of p-phenylenediamines with hydroxy aromatic compounds containing four conjugated double bonds at elevated temperatures in the presence or absence of sodium bisulfite, [Bucherer, J. prakt. Chem. (2) 70, 345 (1904)].

(2) reaction of a primary amino group of a compound containing four conjugated double bonds with a 1-halogen-4-nitro-benzene which may possess a carboxy or sulfo group in the 2-position, and reduction of the nitro group to the corresponding amino, [Goldberg, Ber. 40, 4543, 50 4545 (1907) and German Patent 164,504].

(3) reaction of a halogenated compound containing four conjugated double bonds with a monoacylated p-phenylene-diamine, followed by hydrolysis of the acylated amine.

(4) reaction of a heterocyclic compound containing four conjugated double bonds and a  $-\text{NH}-$  group as a part of the heterocyclic ring, with a nitrobenzene in the presence of alkali, [Helv. Chim. Acta 6, 94-101 (1923)].

Examples of amines of this class prepared by one of the above reactions are as follows:

N-(4-aminophenyl)-1-anthramine



N-(4-aminophenyl)-3-acenaphtheneamine



5

10

15

20

25

30

35

40

45

50

55

60

65

70

75

5-(aminophenylamino)-1,8-naphthosultan



6-(aminophenylamino)-2-methyl-4-phenylquinoline



5-(4-amino-2-carboxyphenylamino)-quinoline-4-carboxylic acid



2-(2-methyl-4-quinolylamino)-5-aminobenzenesulfonic acid



3-(4-aminophenylamino)-9-ethylcarbazole



4-(4-aminophenylamino)-6-methoxyquinoline



5-(aminophenylamino)-1-ethylindole



1-(4-aminophenylamino)-5-benzamidoindole



In the preparation of the diazotype material in accordance with this invention the diazo compound is applied to a suitable carrier such as paper, a regenerated cellulose, cellulose ester or

cellulose ether film, a glass plate, a textile material, a gelatinized surface or metallic surface, by coating or spraying the said carrier with a preparation containing the diazo compound, an azo coupling component such as a phenolic substance, or hydroxy or amino aromatic compound having replaceable hydrogen atoms in the coupling positions which are ortho or para to the directive hydroxy, phenolic or amino groups, or a compound having an active methylene group, a mild acid such as citric or acetic acid, and water. After the selected support or base has been coated by this sensitizing solution, it is dried and exposed under an original positive or negative picture or drawing to a light source emanating light having long wave lengths in the range of 5200-6000 Å, such as a fluorescent light or an incandescent photoflood lamp. It is then developed by contacting the exposed sensitized surface with ammonia vapor or other suitable alkaline materials. As the diluent for the coating solution organic solvents of high volatility such as alcohols, particularly isopropyl alcohol, ethers and ketones, as for example, acetone, may be employed either wholly or partially in place of the water, particularly when the film materials of regenerated cellulose, cellulose esters or cellulose ethers are employed as the carrier.

In another manner of carrying out the process the diazo compound may be added to the coating solution as the only azo dye component and the solution coated onto the carrier in the same manner. The exposure under a suitable positive or negative picture, drawing or the like is effected as before but the image is developed by bathing the exposed element in an alkaline bath containing the azo dye coupler necessary to couple with the undecomposed diazo to form the desired azo dye in the unexposed areas.

As coupling components for the production of the dye image by developing the residual undecomposed diazo compound in the density areas, any compound which will function as a coupling component may be employed either in the coating composition or with the diazo compound as a two-component system or in the developing solution as a color forming developer to be used with a single component diazotype system. In either case, the coupling component selected will be one which will produce the desired color or a combination of coupling components which will produce a desired multi-color effect. Examples of preferred coupling components are the sodium salt of 2-amino-8-naphthol-3,6-disulfonic acid, 2,3-dihydroxynaphthalene or its 6-sulfonic acid or sodium sulfonate derivative,  $\beta$ -naphthol-3,6-disulfonic acid, 2,7-dihydroxynaphthalene, 1,7-aminonaphthol, 2-hydroxynaphthalene-8-bi-guanide, 1-amino-8-naphthol-3,6-disulfonic acid, 1-naphthol-4-sulfonic acid, 1-naphthol-3,8-disulfonic acid, phloroglucinol and resorcinol derivatives such as resorcinol monoacetate, m-hydroxyphenylurea, acetoacetanilide, 7-hydroxy-1,2-naphthamidizole, 7-hydroxynaphthalene-1-bi-guanide and cyclohexyl acetoacetamide.

Although the diazo compounds of this invention are particularly sensitive to long wave light of wave lengths greater than 4200 Å, and as high as 6000 Å, which wave lengths are emitted by fluorescent lights, they are also sensitive to shorter wave length light, and in view of this dual sensitivity as compared with diazo compounds heretofore employed in diazotype production, which latter do not enjoy the long wave sensitivity, the new diazo compounds permit the utilization of

a greater percentage of the total radiation of high pressure quartz mercury arc lamps than the diazo materials which are sensitive only to the shorter wave lengths. This wider utility of the total radiation from such a light source is also due to the fact that the new diazo compounds utilize one of the major emission bands in the green region of the spectrum which is 5400-6000 Å. The net effect of this property of the new diazo compounds is an increased speed of decomposition, or increased printing speed, as compared with diazo compounds heretofore employed when using the high pressure mercury arc lamp as the light source for exposure, which light source is extensively in use. The new diazo compounds therefore have a two-fold advantage over diazo compounds heretofore employed, one being the increased printing speed when using conventional sources of light and the second being the adaptability to sources of light which are poor in short-wave emanations, that is, less than 4200 Å, but rich in long-wave emanations above that band.

The new diazo compounds also have the advantage due to their sensitivity to longer wave length light of producing prints of greater contrast than conventional diazotype materials when used in the intermediate or transition diazotype printing process. In the preparation of intermediate or transition diazotype copies where a diazotype transparency is first produced on transparentized paper or cellulosic film which has been sensitized to produce a dye image highly absorptive of ultraviolet light, a diazo compound which is sensitive to light of a wave length of from 3600-4200 or 4500 Å, is transformed by the usual diazotype methods to an azo dye print having a maximum absorption in the range of 4000-5000 Å. In the printing of further copies from such an intermediate or transition copy better prints are obtained if a diazotype paper can be used which is sensitive to light in the range of 4000-5000 Å, than will be obtained by using a paper sensitive to the range of 3600-4500 Å. The intermediate prints, therefore, which are made with conventional diazotype materials do not efficiently yield diazotype copies with present diazotype materials since the azo dye images of the intermediate print do not efficiently absorb light having the shorter wave lengths and consequently, a portion of the diazo under the dye image is affected. If diazotype papers containing the new diazo compounds of this mention are employed, more satisfactory prints will be obtained in view of the sensitivity of the new diazo compounds to the longer wave length light.

In the following specific examples the preparation of a number of representative diazo compounds of the above class is set forth and the results obtained by using these diazo compounds in typical diazotype coatings are indicated. It is to be understood that these examples are presented as illustrations of the preferred manner of carrying out the invention but not as limitations of its scope. Unless otherwise stated, parts given are by weight.

*Example 1.—4-diazophenyl- $\alpha$ -naphthylamine*



A mixture of 13.5 parts of 4-aminophenyl- $\alpha$ -naphthylamine [prepared by the method of J. prakt. Chem. (2), 60, 557 (1899)], 125 parts water and 18 parts concentrated hydrochloric acid is cooled to 0° C. While the suspension is being agitated, 24 parts of 5 molar sodium nitrite solution is added. The mixture is stirred for 19 hours and filtered. To the filtrate is added 17 parts of an 85% solution of zinc chloride. The brown solid which separates is recovered by filtration. Diazotype coatings of the material in conjunction with resorcinol, 1-phenyl-3-methylpyrazolone and 2,3-dihydroxynaphthalene gave brown, orange and purple prints respectively.

A mixture of 1.0 part of the zinc chloride complex of 4-( $\alpha$ -naphthylamino)-benzenediazonium chloride, 1.5 parts citric acid, 1.5 parts thiourea, 50 parts water and 0.25 part of 3,5-dihydroxybenzoic acid is coated on rag sulfite paper. This coating shows sensitivity to light, having wave lengths between 3250 Å. and 5200 Å. with a maximum sensitivity of 4350 Å. These values may be compared with the sensitivity of p-diethylaminobenzenediazonium chloride complex of zinc chloride, which is sensitive to light in the range of 3500-4600 Å., with a maximum sensitivity at 4100 Å.

*Example 2.—4-diazophenyl- $\beta$ -naphthylamine*



A mixture of 12 parts of p-aminophenyl- $\beta$ -naphthylamine [prepared by the process of J. prakt. Chem. (2), 75, 249-93] is added to a boiling mixture of 190 parts water and 6 parts concentrated hydrochloric acid. To this mixture is added 12 parts of concentrated hydrochloric acid. The mixture is cooled to -3° C. and 40 parts of 5 molar sodium nitrite solution is added. This mixture is stirred for 18 hours and the excess nitrite is destroyed by the addition of urea and the mixture is filtered. To the filtrate is added 10 parts of concentrated hydrochloric acid and 18 parts of an 85% solution of zinc chloride. The mixture is cooled and filtered. A yellow-orange solid, which is recovered, is coated on paper.

Coatings of the diazonium complex with resorcinol, 1-phenyl-3-methylpyrazolone and 2,3-dihydroxynaphthalene gave brown, orange-red and purple prints respectively.

It was found that the 4-( $\beta$ -naphthylamino)-benzenediazonium complex of zinc chloride is light sensitive in the range of 3600-5400 Å. with a maximum sensitivity at 4700 Å.

*Example 3.—2-(p-diazophenylamino)-naphthylene-6-sulfonic acid*



A mixture of 40 parts of 73% pure 2-hydroxynaphthalene-6-sulfonic acid, 120 parts water, 30 parts p-phenylenediamine dihydrochloride and 500 parts sodium bisulfite is heated under reflux for 16 hours; then on a steam bath for an additional 24 hours. The solution is cooled and filtered. Upon drying, a fine powdery solid is obtained.

A mixture of 6.7 parts of 2-(p-aminophenylamino)-naphthalene-6-sulfonic acid, 0.8 part of

70 sodium hydroxide and 90 parts of water are heated to boiling to dissolve the solids. The mixture is cooled and 1 part of concentrated hydrochloric acid is added. To the stirred mixture is added a solution of 2.1 parts sodium nitrite in 5 parts of water. The solution was heated and added dropwise to a mixture of 17 parts of concentrated hydrochloric acid and 2.8 parts of an 85% solution of zinc chloride. This mixture is stirred for 24 hours, cooled and filtered. A black sticky product, upon drying, is converted to a black powdery solid. Diazotype coatings of the diazo complex with resorcinol, phloroglucinol and 2,3-dihydroxy-naphthalene gave brown, brown and purple prints respectively.

A coated paper using diazotized p-aminophenyl- $\beta$ -naphthylamine as the light-sensitive component was exposed beneath a step wedge image in contact with a fluorescent lamp for 2 minutes and developed by the usual methods to yield a satisfactory azo dye image. A standard diazotype paper of the most rapid type required 3½ minutes exposure to the fluorescent lamp to give a comparable print, i. e., the printing speed of the new material is nearly double that of the fastest diazotype material now produced when printed by means of a fluorescent light, as a source of long wave length light.

*Example 4.—N-(p-diazophenyl)-carbazole*



To a hot solution of 29.4 parts of N-(p-aminophenyl)-carbazole [prepared by the method of Helv. chim. Acta 6, 94-101 (1923)] in 300 parts of formic acid (90%) was added 10.1 parts of concentrated hydrochloric acid. On cooling the solution to 10-15° C., a white precipitate was noted. To the suspension at 10° C. was added dropwise, over a period of 45 minutes, 21 parts of 5 molar sodium nitrite solution. A trace of sulfamic acid was added to destroy the excess nitrite. To the mixture was added 320 parts of a 10% solution of naphthalene-1,5-disulfonic acid. A yellowish-brown crystalline solid, amounting to 33 parts, was isolated by filtration. The solid was found to be 93% pure on the basis of a diazo nitrogen analysis. Diazotype coatings of the complex with resorcinol yielded an orange-brown print.

A solution of 1.8 parts of 9-(p-aminophenyl)-carbazole diazonium zinc chloride complex, 5 parts of citric acid and 50 parts of water was coated on rag sulfite paper. This material was found to be sensitive to light having a wave length of 4000-5900 Å with a maximum sensitivity of 4950 Å.

*Example 5.—2-(p-aminophenylamino)-quinoline*



A mixture of 200 parts of 2-chloroquinoline and 150 parts of p-aminoacetanilide is heated gently. The mixture melts at 91-100° C.; then an exothermic reaction causes the temperature to rise to 220° C. The flask is cooled and the mixture allowed to react at 175-195° C. for 15 minutes. The recovered solid mass is ground in a mortar. The

powder is extracted twice with 500 parts of low-boiling ether. The yellow-orange powder, amounting to 324 parts, was probably the mono-hydrochloride of 2-(p-acetamidophenylamino)-quinoline.

A mixture of 3.5 parts of the solid, 50 parts of ethanol, 10 parts of concentrated hydrochloric acid was heated for a few minutes, then filtered to remove insoluble material. The filtrate was refluxed for 2 hours. A crystalline yellow solid separated and was recovered by filtration, then washed with ethanol and ether. This material was shown by analysis to be the dihydrochloride of 2-(p-aminophenylamino)-quinoline.

A mixture of 11.7 parts of 2-(p-aminophenylamino)-quinoline, 50 parts of water and 20 parts of concentrated hydrochloric acid is cooled to 0° C. A solution of 3.5 parts of sodium nitrite and 7 parts of water is added dropwise over a period of 15 minutes and the mixture stirred for an additional 30 minutes. A yellow precipitate, which formed, is dissolved by adding 500 parts of absolute alcohol to the mixture. The mixture is cooled to -10° C. and filtered. The product, amounting to 13 parts, is purified by dissolving 6 parts of the material in 350 parts of water, cooling to 0° C. and adding 40 parts of 85% zinc chloride. The brilliant yellow solid, which formed, is cooled and dried in vacuo.

Coatings of this material with sodium 2-hydroxy-naphthalene-3,6-disulfonate, 2,3-dihydroxynaphthalene and phloroglucinol gave red, brown and yellow diazotype prints respectively.

I claim:

1. A diazotype material comprising an insoluble support having a non-colloidal coating containing a light sensitive diazo derivative of a p-phenylenediamine of the following formulae:



and



wherein R is a member of the group consisting of hydrogen, alkyl, and substituted alkyl; Y is a member of the group consisting of hydrogen, carboxyl and sulfonic acid radicals; R1 is a member of the group consisting of aromatic and heterocyclic radicals of the naphthalene, anthracene,

quinoline, carbazole, and indole series; and R2 is a heterocyclic ring system containing the N atom as a hetero atom selected from the group consisting of indole and carbazole ring systems.

2. A diazotype material comprising an insoluble support having a non-colloidal coating containing as the light sensitive agent a diazo derivative of 4-aminophenyl- $\alpha$ -naphthylamine having the structural formula:

10



and an azo dye coupling component.

15

3. A diazotype material comprising an insoluble support having a non-colloidal coating containing as the light sensitive agent a diazo derivative of 2-(p-aminophenylamino)-naphthylene-6-sulfonic acid having the structural formula:

20

25



and an azo dye coupling component.

30

4. A diazotype material comprising an insoluble support having a non-colloidal coating containing as the light sensitive agent a diazo derivative of N-(p-aminophenyl)-carbazole having the structural formula:

35



40 and an azo dye coupling component.

WILLARD D. PETERSON.

#### REFERENCES CITED

The following references are of record in the file of this patent:

#### UNITED STATES PATENTS

| Number    | Name           | Date          |
|-----------|----------------|---------------|
| 1,756,400 | Schmidt et al. | Apr. 29, 1930 |
| 1,758,676 | Schmidt et al. | May 13, 1930  |
| 1,983,005 | Sakurai        | Dec. 4, 1934  |
| 2,100,063 | Zahn           | Nov. 23, 1937 |
| 2,277,409 | Murray         | Mar. 24, 1942 |